

# UNITED STATES PATENT OFFICE.

ROBERT ADDOTT HADFIELD, OF WESTMINSTER, ENGLAND.

## MANUFACTURE OF MANGANESE-STEEL SHEETS.

1,344,392.

Specification of Letters Patent. Patented June 22, 1920.

No Drawing.

Application filed August 17, 1917. Serial No. 185,520.

To all whom it may concern:

Be it known that I, Sir Robert Addott HADFIELD, baronet, F. R. S., a subject of the King of Great Britain and Ireland, residing at city of Westminster, England, have invented Manufacture of Manganese-Steel Sheets, of which the following is a specification.

This invention has for object to produce thin steel sheets that shall be specially suitable for use as a protective material against bullets, shrapnel and the like and which shall offer greater resistance to perforation and fracture by missiles of the kind referred to than steel sheets of the same thickness heretofore produced and which shall therefore be specially adapted for use in the manufacture of helmets, body shields, and the like for the use of soldiers and others engaged in war, as protective sheeting for use in air craft and for like protective purposes but suitable also it may be for other purposes.

The invention also has for object to produce sheet steel helmets made of such sheet protective steel.

For attaining the above mentioned objects, sheet steel according to this invention and specially adapted for purposes such as set forth, is made of steel of the kind known as Hadfield's manganese steel, comprising iron with from 10 to 17 per cent. of manganese and carbon up to about two per cent. but usually from about .9% to 1.3% or 1 to 2% and also it may be other elements, for instance silicon or copper, or silicon and copper, as described in the specification of my applications for Letters Patent, Serial No. 185,521 filed August 10th, 1917, Serial No. 103,995 filed July 18th, 1916, and Serial No. 109,436, filed July 15th, 1916.

For the manufacture of thin sheets of manganese steel capable of offering great resistance to perforation and fracture by missiles such as those hereinbefore referred to and therefore suitable for use as a protective material for purposes such as set forth, such steel owing to its peculiar characteristics, must be produced and treated in a special way in order that it shall have imparted to it the necessary qualities of hardness and toughness to render it possible to be successfully used for the purposes mentioned. Thus, manganese steel of the kind hereinbefore mentioned and made for

instance by the addition of ferro-manganese to decarbonized, demanganized and desilicized iron in known manner, must be cast in such a way as to produce perfectly sound ingots, that is to say, ingots free from piping and segregation, as for instance by pouring the molten manganese steel into ingots and allowing the ingots to cool from the bottom upward and maintaining the upper portion of the metal in a molten state, as by applying heat thereto, until the lower portion of the metal has solidified, so that such upper molten metal can descend and compensate for shrinkage of the metal, due to cooling, and thus prevent piping and segregation that would otherwise occur, and thus enable sound metal ingots to be obtained so that when converted into the form of thin sheets, such sheets shall be free from unsoundness.

For converting a sound manganese steel ingot thus produced into sheets possessing great hardness and toughness and therefore resistance to perforation and fracture, the ingot is first converted, while at a high temperature into a slab, as by hammering, pressing or rolling it and the resulting slab is cut into lengths suitable for the convenient production of steel sheet of the desired thickness. Satisfactory results have been obtained by maintaining the metal at an average forging temperature of the order of about 1050° to 1080° C. during its conversion into the form of a slab.

After cooling, the resulting slab is carefully examined and all laminations or surface imperfections removed by grinding or otherwise, as well as any split ends on the slab.

The clean slab thus obtained is afterward cut into shorter slab lengths each heated and which is converted by rolling into steel sheets of the required thickness. This is done by a succession of rolling operations each designed to reduce the thickness of the metal to a suitable degree and thus prevent undue compression of the metal, at any one stage of reduction, that might injuriously affect the desired qualities of the required finished steel sheets the temperature of rolling being high. Satisfactory results have been obtained when using a rolling temperature of the order of about 1080 to 1040° C., the temperature of the finished sheet obtained by the last rolling operation being 110

preferably about 850° C. Great care should be taken during the heating of the slab and resulting plates and sheets, preparatory to the several rolling operations, to avoid, as much as possible, oxidation of such plates and sheets.

5 The manganese steel sheets thus obtained must then be annealed in a non oxidizing atmosphere, to remove therefrom the hardness caused by the later stages of the rolling.

10 The annealed steel sheets are then cut or stamped into sheets of the size required for conversion into helmets, body shields or other articles. Such sheets are afterward 15 carefully subjected to further heat treatment and water toughened. For this purpose they are first heated rapidly and equally to a high temperature, the heating being carried out in such a manner as practically to avoid oxidation of the sheets. For 20 this purpose the sheets may be supported singly above the floor of a reheating furnace, as for instance upon small iron bars placed on such floor, the furnace being so fired and worked that practically a neutral or non-oxidizing atmosphere is maintained therein. For this purpose a gas or oil fired furnace is preferred. The sheets after being thus equally heated are removed from the 25 furnace and at once quenched in a cold liquid while at a high temperature. Satisfactory results have been obtained by quenching the sheets while at a temperature of the order of about 950° to 1050° C., preferably 30 at about 1000° C., in cold water. The whole 35 operation of heating preparatory to quenching, should not occupy more than about two or three minutes.

40 The manganese steel sheets thus produced are then in a condition ready to be converted into a helmet or other article of the required shape, as by stamping or pressing.

45 The following is a detailed description, given by way of example only, of a method whereby sound manganese steel ingots produced as described, have been converted into thin metal sheets and such sheets converted into helmets that have been found by severe tests to give highly satisfactory results in 50 practice, as regard hardness and toughness and consequent resistance to perforation and fracture.

55 The manganese steel contained about 1.25% to 1.4% of carbon and about 13.0% to 13.75% of manganese. The ingots were of taper shape, cast with their larger ends upward and in the manner hereinbefore described to produce sound steel ingots, each ingot being about 9" square and weighing 60 about 10 to 10.5 cwts. Each ingot was hammered or pressed at a forging temperature of about 1050° to 1080° C. into a slab 7" wide and 2" thick and then cut into shorter slab lengths each having a weight of about 65 56 lbs., the metal being heated twice to about

the forging temperature hereinbefore mentioned, namely 1050° to 1080° C., to enable it to be properly converted from the ingot form into the finished slab.

70 Each of the short slab lengths having a width of 7" and thickness of 2" was then converted into sheet form by subjecting it to four successive heating and rolling operations as follows:

75 *First operation.*—The slab was reheated to a rolling temperature of about 1030° to 1040° C. and rolled down into a plate or bar 9" wide and  $\frac{1}{8}$ " thick, which was then cut into six pieces each about 15" in length.

80 *Second operation.*—Each of the said plates was then reheated to a rolling temperature of about 1030° C. and rolled "long-way on" into a sheet 18" to 20" in length, 15.75" wide and about .05" thick.

85 *Third operation.*—The sheets thus produced were reheated in pairs to a temperature of about 1030 C. and after removing all scale therefrom, were rolled in pairs.

90 *Fourth operation.*—Each sheet was then again reheated and rolled so as to produce a sheet about 50" long, 15.75" wide and of a thickness of about .086" that is to say, of No. 20 gage, the finishing temperature of the sheet being about 850° C. During each reheating, great care was taken to avoid, as far as possible, oxidation of the sheets, by 95 maintaining a non oxidizing atmosphere in the reheating furnace.

100 Out of each of the rolled sheets thus produced, three disks, each 14.25" in diameter were stamped, each disk being suitable for one helmet.

105 Before being divided by stamping into helmet blanks, the rolled sheets, were, in order to remove therefrom the hardness caused by the later stages of the rolling, annealed, as by introducing them into a furnace, such as a mill furnace, and heating them to a temperature of about 700 to 750° C., after which they were taken out of the 110 furnace and cooled in piles.

115 From the annealed sheets circular sheets were stamped to form the helmet blanks. The helmet blanks were heated separately and equally in a non-oxidizing atmosphere to a high temperature in a gas fired furnace for two or three minutes and withdrawn from the furnace at a temperature of from 950° to 1050° C., but preferably about 1000° C., and quenched in cold water, this forming the heat treatment and toughening treatment of the sheets hereinbefore described.

120 The circular helmet blanks were then placed in a press and stamped in a die to the desired finished shape for instance that of a concave circular or oval bowl or dish. To enable this to be done successfully, it is necessary that each circular steel sheet blank should be flat and the edge portion thereof 125

lubricated all around before putting it into the press and care must be taken to obtain a very even bearing for the sheet on the die before the pressing to shape takes place 5 otherwise distortion of the sheet will result.

Instead of stamping circular blanks out of the rolled sheet the latter may be cut into square or rectangular sheets and heat treated and toughened as described, such sheets 10 being afterward stamped to the circular or other desired shape as and where required for conversion into helmets or other articles.

What I claim is:—

1. The manufacture of sheet manganese steel which consists in gradually reducing 15 a slab of manganese steel by a succession of rolling operations while at a suitable forging temperature into a sheet of the desired thickness and so that the temperature of 20 the sheet at the last rolling operation is of the order of about 850° C., annealing the resulting sheet, heating the annealed sheet rapidly and equally and for a short time only, to a high temperature and then plunging 25 it into a cold liquid.

2. The manufacture of manganese steel sheets suitable for use as a protective material as set forth, which consists in casting a sound ingot of manganese steel, converting 30 such ingot into a billet or slab while at an average temperature of about 1050° to 1080° C., cutting said slab into shorter slab lengths, gradually reducing such slab lengths while at a suitable forging temperature 35 into sheets of the desired thickness, annealing the resulting sheets, heating the annealed sheets rapidly and equally and for a short time only to a high temperature and then cooling them suddenly.

40 3. The manufacture of manganese steel sheets suitable for use as a protective material as set forth, which consists in casting a sound ingot of manganese steel, converting such ingot into a billet or slab at an 45 average temperature of about 1050° to 1080° C., cutting said slab lengths into shorter slab lengths, gradually reducing said slab lengths by rolling into sheets of the desired thickness at a temperature of about 1030° 50 to 1040° C., annealing said sheets and subjecting the annealed sheets to a heat treatment and to a water toughening treatment consisting in heating them to a high temperature for a short time only and suddenly cooling them by immersion in cold 55 liquid.

4. The manufacture of thin manganese steel sheets, suitable for use as a protective material as set forth, which consists in casting 60 a sound ingot of manganese steel, converting said ingot at an average forging temperature of about 1050° to 1080° C. into a slab and cutting said slab into shorter slab lengths, rolling each slab length of metal 65 into a sheet of the desired thickness by a

succession of rolling operations, the metal at the commencement of each rolling operation being at a temperature of about 1030° to 1040° C. and after rolling, except the last one, being reheated to a temperature of 70 about 1030° C. to 1040° C., the finishing temperature of the sheet, after the last rolling 75, being about 850° C., annealing the resulting sheet, heating the annealed sheet rapidly and equally to a temperature of about 950° to 1050° C. and then plunging it while at about this temperature into a cold liquid, the duration of such heat treatment of the sheets being of the order of about a few minutes.

5. The manufacture of thin manganese steel sheets, suitable for use as a protective material as set forth, which consists in gradually rolling a plate or slab into a sheet of the desired thickness by a succession of rolling operations, the metal at the commencement of such rolling operation being at a temperature of about 1030° to 1040° C., and after rolling, except the last one, being reheated to a temperature of about 1030° C. 85 to 1040° C., the finishing temperature of the sheet, after the last rolling, being about 850° C., annealing the resulting sheet, heating the annealed sheet rapidly and equally to a high temperature for a short time only and then 90 plunging it while at a high temperature into a cold liquid.

6. The manufacture of thin manganese steel sheets, suitable for use as a protective material as set forth, which consists in gradually converting a plate or slab of manganese steel into a sheet of the required thickness and size by a series of rolling operations with intermediate reheating operations, the average rolling temperature being 105 of the order of about 1030° to 1040° C. and the finishing temperature after the last rolling 100 operation being about 850° C., annealing the resulting sheet, reheating the annealed sheet rapidly and equally for a few minutes 110 to a temperature of the order of about 950° to 1050° C. and then plunging it while at about this temperature into cold water.

7. The manufacture of a thin manganese steel blank, suitable for use as a protective 115 device as set forth, which consists in converting a plate or slab of manganese steel into sheet form by a series of rolling operations with intermediate reheating operations, the average rolling temperature being of the 120 order of about 1030 to 1040° C. and the finishing temperature after the last rolling operation, being about 850° C., annealing the resulting sheet, cutting a blank of the desired size and shape from the annealed 125 sheet, reheating the annealed sheet metal blank, rapidly and equally for a few minutes only to a temperature of the order of about 950° to 1050° C., then plunging it while at about this temperature into cold 130

water, and forming the resulting blank into an article of the desired shape by pressure.

8. The manufacture of a thin manganese steel blank, suitable for use as a protective material as set forth, which consists in gradually reducing a plate or slab of manganese steel by successive rolling operations and while at an average temperature of about 1030 to 1040° C. into a sheet of the desired thickness and size, annealing the resulting sheet, cutting a blank of the desired shape and size from the annealed sheet, heating the annealed sheet metal blank rapidly and equally to a temperature of the order of

about 950 to 1050° C., for a short time only, 15 then plunging it while at about the said temperature into a cold liquid, lubricating the edge portion of the resulting toughened blank and pressing the said blank, while supported evenly, into the shape of the desired article. 20

Signed at 22 Carlton House Terrace, in the city of Westminster, England, this twelfth day of July, 1917.

ROBERT ABBOTT HADFIELD.

Witnesses:

WILLIAM CROSS,  
LEONARD ROWLAND.